

Patented Mar. 7, 1933

1,900,182

# UNITED STATES PATENT OFFICE

DANIEL D. JACKSON, OF BROOKLYN, NEW YORK, ASSIGNOR TO REMINGTON ARMS COMPANY, INC., A CORPORATION OF DELAWARE

## METALLIC ALLOY

No Drawing.

Application filed November 28, 1930. Serial No. 498,755.

This invention relates to alloys, particularly alloys of the type containing substantial percentages of lead, and has for its object the production of an alloy of lead which, while serving the same purpose as other lead alloys, is of a non-poisonous character.

In one aspect the invention contemplates the provision of a non-poisonous lead alloy suitable for use as shot. It is well known that substantial numbers of wild birds, particularly wild fowl, are annually destroyed by lead poisoning. Where extensive shooting occurs for a period of years over the feeding grounds of wild fowl, quantities of lead shot are accumulated and these shot are swallowed by the fowl in the same manner as gravel or any other small hard objects. The shot remain for some time in the gizzard of the fowl and are discharged to the intestine in minute fragments as they are ground up by their own abrasive action. The poisoning effect of such lead particles is known to be due to the formation by the digestive fluids of soluble lead salts which are assimilated and have a very detrimental effect upon certain tissues.

The present invention comprises the discovery of an alloy which, while it consists chiefly of lead and possesses the same characteristics which adapt lead for many different uses, is nevertheless non-poisonous in character. Actual experiments with this alloy upon wild ducks have shown it to be harmless, whereas ordinary lead shot are definitely and certainly poisonous. The alloy comprises an ingredient which has the effect of rendering inactive the salts which are produced by digestive fluids. Just how this effect is produced is not definitely known. It may be that the salts of lead are in some way rendered insoluble, or that different harmless or insoluble salts are formed, or that the alloy is not attacked by digestive fluids. Whatever the theoretical explanation, a surprisingly small amount of the proper ingredient

is sufficient to render shot non-poisonous, this effect being analogous to the effect produced upon the physical and chemical properties of other metals and alloys by the admixture of a small quantity of a particular ingredient or slight variations in the proportions of the ingredients.

One ingredient which thus has the effect of rendering shot harmless to wild fowl is phosphor tin, an alloy consisting of tin with 4% or 5% of phosphorus. An excess of phosphorus is used to compensate for oxidation during the pouring of the shot. Non-poisonous shot are secured by adding .3% to 1% of such phosphor tin to an alloy in current use. For example, a typical non-poisonous shot metal is prepared with the following composition.

|              | Per cent |
|--------------|----------|
| Lead         | 96.5     |
| Arsenic      | .5       |
| Antimony     | 3.0      |
| Phosphor tin | .3       |

This composition is subject to substantial variation, formulas containing up to 1% of phosphor tin having been found to be successful. In the melting of the material for pouring shot some phosphorus and a small proportion of tin is oxidized and lost; the phosphor tin content of the best shot produced varies from .1% to .2%.

It is believed that the present invention comprises the first discovery of the non-poisonous character of such a lead alloy. Accordingly, the appended claims are to be broadly construed.

### What is claimed is:

1. As an article of manufacture, lead shot which has been rendered non-poisonous to animals by the incorporation therein of phosphor tin.
2. As an article of manufacture, shot which is non-poisonous to animals and comprises lead alloyed with .10% to 1% of phosphor tin.

3. As an article of manufacture, lead shot containing a quantity of phosphor tin, whereby the salts produced by the action of the digestive fluids of animals upon the shot are rendered non-poisonous.

4. As an article of manufacture, shot which is non-poisonous to animals and comprises lead, antimony and phosphor tin.

5. As an article of manufacture, shot which is non-poisonous to animals and comprises 95% to 96.5% lead, 3% to 4% antimony, and .1% to 1% of phosphor tin.

DANIEL D. JACKSON.

15

20

25

30

35

40

45

50

55

60

65